

[54] FLOTATION RECOVERY OF  
MOLYBDENITE

[75] Inventors: **Joseph Floyd Shirley**, Tucson, Ariz.;  
**Edward Frank Caropreso**,  
Hightstown, N.J.; **George Lamar**  
**Fraser**, Magna, Utah

[73] Assignee: **FMC Corporation**, New York, N.Y.

[22] Filed: **June 7, 1971**

[21] Appl. No.: **150,773**

[52] U.S. Cl. .... **209/167**

[51] Int. Cl. .... **B03d 1/06**

[58] Field of Search..... **209/166, 167**

## [56] References Cited

## UNITED STATES PATENTS

|           |         |                    |           |
|-----------|---------|--------------------|-----------|
| 2,608,298 | 8/1952  | Arbiter .....      | 209/167   |
| 2,620,068 | 12/1952 | Allen .....        | 209/167   |
| 2,811,255 | 10/1957 | Nokes .....        | 209/167   |
| 3,137,649 | 6/1964  | De Benedictis..... | 319/167 X |

|           |         |              |           |
|-----------|---------|--------------|-----------|
| 3,313,412 | 4/1967  | Bloom.....   | 209/167   |
| 3,220,551 | 11/1965 | Moyer.....   | 209/167   |
| 3,372,924 | 4/1968  | Corbett..... | 209/167   |
| 3,539,002 | 11/1970 | Last .....   | 209/167 X |

Primary Examiner—Robert Halper

## [57] ABSTRACT

A process for separating molybdenite from copper concentrates containing copper and iron sulfides, gangue materials and an organic collector comprising (1) conditioning the concentrate in aqueous suspension at a pH below about 7 with a soluble metal salt; (2) contacting the so treated concentrate with hydrogen peroxide at pH of about 4 to about 8; (3) subjecting the concentrate from (2) to a soluble iron cyanide and/or a solution of phosphorus pentasulfide in sodium hydroxide while maintaining the pH at no higher than about 8.5 whereby the molybdenite is floated and (4) recovering the enriched molybdenite float.

14 Claims, No Drawings

## FLOTATION RECOVERY OF MOLYBDENITE

## BACKGROUND OF THE INVENTION

## 1. Field of the Invention

This invention relates to sulfide ores, particularly to the recovery of molybdenite from flotation concentrates containing a minor amount of molybdenite relative to other metal sulfides.

## 2. Description of the Prior Art

The mineral molybdenite is a naturally occurring molybdenum sulfide ( $MoS_2$ ) and is the principal ore from which metallic molybdenum is obtained. Molybdenite commonly occurs as a minor component in ores containing other metallic sulfides and is recovered therefrom as a by-product in the refining of copper ores by froth flotation. This is a widely used mining technique for the separation of minerals from their ores based on the differential wetting of the particles of finely ground ore.

In the recovery of molybdenite by froth flotation, it is common practice to start with mill concentrates or copper concentrates as they are more often called. These are partially refined sulfide ores from which much of the gangue material has been removed by froth flotation. Mill concentrates usually contain about 15 to about 30 percent copper while the molybdenite assay is typically of the order of 0.2 to 3 percent; other sulfides such as iron sulfide as well as some non-sulfide components may be present.

Since mineral separation by froth flotation depends on the difference in wetting properties of the mineral and ore particles, it is desirable to enhance such differential wetting by means of various collectors and/or depressant agents. Thus, where molybdenite is recovered from copper concentrates, the most common practice is to depress the associated copper and iron minerals while the molybdenite is floated off therefrom using a liquid hydrocarbon, for example, as a smearing collector for the molybdenite.

Accordingly, it is necessary to remove the previously added collectors from the copper and iron sulfide minerals in order to facilitate a separation. One approach to this problem has been the simple addition of a depressant to displace the organic collector from the copper and iron sulfide mineral surfaces. For instance, U.S. Pat. No. 2,492,936 to Nokes et al. discloses several reagents which can be used for this purpose. However, because rather large addition rates of these chemicals are required to obtain satisfactory results, the process is uneconomical where the molybdenite content is relatively low. In U.S. Pat. No. 2,664,199 to Barker et al., sodium ferrocyanide is used to depress copper and iron sulfide minerals after previous conditioning with mild acid. Although this procedure has worked reasonably well in the treatment of chalcocite concentrates, it is generally unsatisfactory when treating concentrates containing predominantly chalcopyrite.

Another approach to separating molybdenite from copper concentrates has been to destroy or chemically alter the previously added copper collectors. This is accomplished in U.S. Pat. No. 2,255,776 to Janney et al. by various heat treatments. For instance, steaming is quite effective for removing xanthate type collectors from copper concentrates containing primarily chalcocite, but gives poor results with copper concentrates containing predominantly chalcopyrite. Moreover, the

process is less than satisfactory in treating copper concentrates containing chalcocite and/or chalcopyrite where a thiophosphate has been used as a collector. Still another modification employs mild roasting which

5 depresses the copper and iron sulfide minerals by oxidizing their surfaces and burning off the previously added collectors. However, the molybdenite is also oxidized to some extent thereby causing it to be depressed. Generally, this procedure has not been used as the primary means of separating molybdenite from copper concentrates due to the relatively high capital investment required. In U.S. Pat. No. 2,559,104 to Arbiter et al. it is suggested that by treating the copper concentrates with an oxidizing agent the copper collectors can 10 be destroyed or altered to lose their collecting ability. As a result the copper and iron sulfide minerals are said to be depressed. Although reasonably successful with copper concentrates containing primarily chalcocite, the procedure does not work satisfactorily on concentrates containing primarily chalcopyrite.

In a more recent patent, namely U.S. Pat. No. 3,137,649 to DeBenedictis et al., copper concentrates are subjected to oxidative treatment with hydrogen peroxide under rigidly controlled conditions of time 15 and pH. The conditioned pulp is then given a froth flotation treatment in the presence of iron cyanide as a depressant. The process is effective in treating copper concentrates which have been collected with a xanthate type collectors, but it has failed to treat satisfactorily copper concentrates collected with a thiophosphate.

Although the aforescribed processes exhibit varying degrees of efficiency, they have not proved to be entirely satisfactory for one reason or another. As a 25 consequence, the art is still seeking further advances in the conditioning of copper concentrates for the purpose of effecting separation of molybdenite from accompanying sulfide ores.

## SUMMARY OF THE INVENTION

It has now been discovered that molybdenite can be separated from copper concentrates recovered by means of organic collectors and containing primarily copper and iron sulfide minerals as well as various gangue materials by (1) conditioning such concentrates with a soluble metal salt at a pH below about 7; (2) subjecting the so treated concentrates to a second conditioning with an oxidant; (3) subjecting the so conditioned concentrate to a depressant system which selectively depresses the molybdenite fraction and (4) subjecting the molybdenite to froth flotation to recover the enriched molybdenite float.

## GENERAL DESCRIPTION

55 In accordance with the invention, copper concentrate (usually containing 0.25-2.0 percent molybdenite and about 25 percent copper or iron in the form of a mixed sulfide) may be treated as it comes from the copper concentration plant or it may be thickened to contain 40-60 percent solids. Treatment in the first conditioning step consists of adding fuel oil and a solution containing the dissolved metal salt. Acid is also added at this point for pH control or adjustment. The pulp is 60 next treated in a second conditioning tank with an oxidant preferably hydrogen peroxide or another peroxy- 65 gen compound and again adjustment of the pH with acid or base may be necessary. The pulp is next treated

with a depressant or depressants before it enters the rougher flotation cells. Since the various depressants require different conditions for satisfactory operation, the pH of the pulp at this point will be dictated by the choice of depressant or depressants.

The copper concentrate may contain 16-60 percent solids although we prefer to work at 40-60 percent solids. Less reagents are required at the higher pulp densities and thus should be as high as possible in the interest of low operating costs.

The amount of fuel oil required to produce a hydrophobic surface on the molybdenite will depend on the ore. Usually 0.1-1.0 lb. of fuel oil per ton of concentrate is sufficient. It is preferred that the fuel oil be added prior to addition of oxidant.

Sufficient metal salt should be added to react with all or most of the collector which is contained in the copper concentrate. Normally, 0.5-3.0 lb. of metal salt per ton of concentrate is satisfactory.

So far as we have been able to ascertain, any soluble metal salt capable of reacting or complexing with the dithiophosphate or the products of the reaction of the oxidant with the dithiophosphates can be used. However, it has been our experience that soluble metal sulfates particularly cupric sulfate, aluminum sulfate, and/or zinc sulfate provides reproducible and highly satisfactory results at low cost.

During the first conditioning step, pH control is not particularly critical. However, it is desirable to adjust the pH to about 5.5-7.5 so as to provide suitable conditions for the oxidant reaction in the second conditioning step.

Temperature and time do not appear to be critical factors during the first conditioning operation.

Following the first conditioning operation the oxidant is added. The amount of oxidant is dependent on the ore, the type of oxidant, the slurry density, the type and amount of dithiophosphate used as collectors and the particular depressant or depressants used in the subsequent rougher flotation circuit. So far as we have been able to ascertain, any number of oxidants are suitable although we prefer peroxygen compounds such as ammonium and alkali metal persulfates, sodium permonosulfate, alkali metal peroxides or hydrogen peroxide, the latter being especially preferred.

Broadly, we have found that the process disclosed in the invention can be carried out using about 0.25 to about 4 lbs. of hydrogen peroxide per ton of concentrate, although the preferred range is about 0.5-2 lbs. per ton of concentrate. The reaction between the dithiophosphate, metal ion and hydrogen peroxide occurs rather rapidly between a pH of about 4 and 8 whereas outside this range the reaction proceeds more slowly. Optimum pH range is in the vicinity of 5.5-7.5.

After the hydrogen peroxide addition, the pH of the pulp is adjusted to provide proper conditions in the rougher flotation cells. Thus, in order that the ferrocyanide function satisfactorily as a depressant, the pH should be between 6.5 and 8.5 and therefore the pulp pH should be less than 8.0. The reason for operating below pH 8 is that ferrocyanide reacts with excess  $H_2O_2$  and converts a portion of the ferrocyanide to ferricyanide. This reaction results in an increase in pH. There-

fore, to achieve the requisite condition in the rougher circuit the pulp should be below pH of 8.0.

One of the particularly desirable aspects of the present process is that it effects separation of molybdenite from most iron and copper sulfide minerals including the difficult pyrite and chalcopyrite types and, of course, as well as the more easily treated chalcocite ores. Moreover, the process is effective in removing dithiophosphate collectors which are stable and difficult to destroy. It is to be pointed out that if copper sulfate is the metal salt chosen the copper sulfate and part of the acid used in the first conditioning step can come from copper leach solutions which are available at most mills. Thus, the copper values from these leach solutions can be recovered easily and economically since the copper in the process eventually ends up in the smelter in any event. Normally, the copper in leach solutions is recovered by precipitation, so the present process effects its precipitation using chemicals already in the circuit. Where sulfide type depressants e.g. sodium sulfide,  $(Na_2S)$  sodium hydrosulfide ( $NaHS$ ) are used in the molybdenite recovery circuit, their requirement will be greatly reduced from what it would be if the copper concentrates were not pre-conditioned with copper sulfate and hydrogen peroxide in accordance with the invention.

Reference is now made to the following non-limiting examples.

### Experimental Procedure

### MATERIALS

The copper concentrates consisted primarily of chalcocite and pyrite with minor amounts of chalcocite, bornite, molybdenite and talc. The major collector used to promote the copper minerals in these concentrates was either a mixture of  $P_2S_5$  and cresylic acid or Aerofloat 238, a product of American Cyanamid reported to be sodium di-secondary butyl dithiophosphate. Two batches of concentrates were processed having the following assay:

Series A - 1.56%  $MoS_2$ , 27.3% Cu  
Series B - 2.85%  $MoS_2$ , 32.3% Cu

### REACTION CONDITIONS

A. 8-15 minutes with the indicated quantity of metal sulfate, and 0.033 lb/ton of fuel oil at a pH of 6.5.  
B. Treatment for 5 minutes with hydrogen peroxide at pH 6.5.  
C. Sodium ferrocyanide and/or a Nokes reagent (13 parts  $NaOH$  to 10 parts  $P_2S_5$ ) were then added as depressants. When used in combination, the sodium ferrocyanide was added first and allowed to mix for 1 minute before addition of the Nokes reagent. Approximately 0.165 lb/ton of methyl amyl alcohol frother was also added.

D. The conditioned pulp was floated for 6 minutes at a final pH ranging from 7.7 - 8.0. The molybdenite was then separated as an enriched float in the rougher.

The individual examples are summarized in the Table below.

| Example No. | Conditioning agents                                   |           | Depressant system             |                                     |                                                  | Percent wt. floated | Concentrate      |              | Tailing          |              |                  |       |      |      |
|-------------|-------------------------------------------------------|-----------|-------------------------------|-------------------------------------|--------------------------------------------------|---------------------|------------------|--------------|------------------|--------------|------------------|-------|------|------|
|             | Metal sulfate                                         |           | H <sub>2</sub> O <sub>2</sub> | Na <sub>4</sub> Fe(CN) <sub>6</sub> | P <sub>2</sub> S <sub>5</sub> /NaOH <sup>1</sup> |                     | Assay percent    | Distribution | Assay percent    | Distribution |                  |       |      |      |
|             | Name                                                  | lb/ton    | lb/ton                        | lbs/ton                             | lbs/ton                                          |                     | MoS <sub>2</sub> | Cu           | MoS <sub>2</sub> | Cu           | MoS <sub>2</sub> | Cu    |      |      |
| 1A.....     | CuSO <sub>4</sub> - 5H <sub>2</sub> O.....            | 2.0 ..... | .....                         | 0.8                                 | 1.25                                             | 91.32               | .....            | .....        | .....            | .....        | .....            | ..... |      |      |
| 2A.....     | .....                                                 | 1.25      | .....                         | .8                                  | .....                                            | 89.75               | .....            | .....        | .....            | .....        | .....            | ..... |      |      |
| 3A.....     | .....                                                 | 1.25      | .....                         | .....                               | 1.25                                             | 88.10               | .....            | .....        | .....            | .....        | .....            | ..... |      |      |
| 4A.....     | .....                                                 | 1.25      | .....                         | .8                                  | 1.25                                             | 88.72               | .....            | .....        | .....            | .....        | .....            | ..... |      |      |
| 5A.....     | CuSO <sub>4</sub> - 5H <sub>2</sub> O.....            | 2.0       | 1.0                           | .....                               | .....                                            | 85.95               | 1.64             | 28.2         | 94.2             | 93.2         | 0.62             | 12.7  | 5.9  | 6.8  |
| 6A.....     | CuSO <sub>4</sub> - 5H <sub>2</sub> O.....            | 2.0       | 1.0                           | 1.6                                 | .....                                            | 73.19               | 2.06             | 29.6         | 96.2             | 81.5         | .22              | 18.4  | 3.8  | 18.5 |
| 7A.....     | CuSO <sub>4</sub> - 5H <sub>2</sub> O.....            | 2.0       | 1.0                           | .....                               | 1.25                                             | 24.29               | 6.35             | 27.1         | 94.4             | 25.0         | .12              | 26.1  | 5.6  | 75.0 |
| 8A.....     | CuSO <sub>4</sub> - 5H <sub>2</sub> O.....            | 2.0       | 1.0                           | 0.8                                 | 1.0                                              | 19.60               | 7.3              | 27.1         | 89.0             | 20.6         | .22              | 25.4  | 11.0 | 79.4 |
| 9A.....     | ZnSO <sub>4</sub> - 7H <sub>2</sub> O.....            | 3.2       | 1.0                           | .8                                  | 1.25                                             | 14.80               | 9.4              | 25.6         | 90.1             | 14.5         | .18              | 26.3  | 9.9  | 85.5 |
| 10A.....    | Al <sub>2</sub> (SO <sub>4</sub> ) <sub>3</sub> ..... | 4.0       | 1.0                           | .8                                  | 1.25                                             | 13.70               | 9.7              | 27.0         | 84.6             | 14.0         | .28              | 26.4  | 15.4 | 86.0 |
| 1B.....     | ZnSO <sub>4</sub> - 7H <sub>2</sub> O.....            | 3.2       | 0.5                           | .8                                  | 0.94                                             | 11.50               | 14.2             | 28.6         | 73.6             | 10.4         | .66              | 31.9  | 26.4 | 89.6 |
| 2B.....     | ZnSO <sub>4</sub> - 7H <sub>2</sub> O.....            | 3.2       | .7                            | .8                                  | 1.15                                             | 12.80               | 12.6             | 25.1         | 81.5             | 11.0         | .42              | 29.6  | 18.5 | 89.1 |
| 3B.....     | ZnSO <sub>4</sub> - 7H <sub>2</sub> O.....            | 3.2       | 1.0                           | .8                                  | 1.15                                             | 5.90                | 33.2             | 17.0         | 91.3             | 3.2          | .20              | 32.6  | 8.7  | 96.8 |
| 4B.....     | ZnSO <sub>4</sub> - 7H <sub>2</sub> O.....            | 3.2       | 1.0                           | .8                                  | 0.94                                             | 12.05               | 15.0             | 25.3         | 63.9             | 9.9          | 1.16             | 31.7  | 36.1 | 90.1 |
| 5B.....     | ZnSO <sub>4</sub> - 7H <sub>2</sub> O.....            | 3.2       | 1.0                           | .8                                  | 1.25                                             | 6.20                | 37.5             | 13.3         | 87.9             | 2.6          | 0.34             | 32.7  | 12.1 | 97.4 |
| 6B.....     | ZnSO <sub>4</sub> - 7H <sub>2</sub> O.....            | 3.2       | .....                         | .8                                  | 1.25                                             | 6.80                | 21.7             | 22.8         | 60.7             | 4.9          | 1.02             | 32.2  | 39.3 | 95.1 |

<sup>1</sup> Lbs/ton values based on P<sub>2</sub>S<sub>5</sub> added.

## Analysis of Test Data

The data summarized in the Table show:

1. The necessity for conditioning with both a metal sulfate and H<sub>2</sub>O<sub>2</sub> before flotation. This was demonstrated by the observation that the following reagent schedules were ineffective for separating MoS<sub>2</sub> from copper concentrates promoted with dithiophosphate type collectors.
  - a. H<sub>2</sub>O<sub>2</sub> - Na<sub>4</sub>Fe(CN)<sub>6</sub>
  - b. H<sub>2</sub>O<sub>2</sub> - P<sub>2</sub>S<sub>5</sub>/NaOH
  - c. H<sub>2</sub>O<sub>2</sub> - Na<sub>4</sub>Fe(CN)<sub>6</sub> - P<sub>2</sub>S<sub>5</sub>/NaOH
  - d. CuSO<sub>4</sub> - Na<sub>4</sub>Fe(CN)<sub>6</sub> - P<sub>2</sub>S<sub>5</sub>/NaOH
2. That several depressant systems are applicable, e.g. sodium ferrocyanide, Nokes reagent (mixture of P<sub>2</sub>S<sub>5</sub>/NaOH), and mixtures of the two. Best results with respect to physical characteristics and metallurgical analysis were obtained using the combination of reagents.
3. That metal sulfates such as CuSO<sub>4</sub>, ZnSO<sub>4</sub>, and Al<sub>2</sub>(SO<sub>4</sub>)<sub>3</sub> may be used. When using the combination depressant system Na<sub>4</sub>Fe(CN)<sub>6</sub> and P<sub>2</sub>S<sub>5</sub>/NaOH, the ZnSO<sub>4</sub> gave the better results.
4. The dependence of MoS<sub>2</sub> separation upon H<sub>2</sub>O<sub>2</sub> usage - metallurgical results improved with increasing quantities of H<sub>2</sub>O<sub>2</sub>.
5. At constant sodium ferrocyanide usage, improved metallurgical results are obtained by using increasing amounts of the P<sub>2</sub>S<sub>5</sub>/NaOH mixture.

What is claimed is:

1. In a process for the separation of molybdenite from copper concentrates obtained by froth flotation in the presence of an organic collector, the improvement whereby the molybdenite is recovered in a more concentrated form comprising:
  1. conditioning the concentrate in aqueous suspension at a pH below about 7 with a water soluble metal salt of copper, zinc or aluminum;
  2. contacting the so-treated concentrate with an oxidant selected from the group consisting of hydrogen peroxide, sodium peroxide, ammonium, alkali metal persulfate and sodium permonosulfate;
  3. subjecting the so conditioned concentrate to a depressant selected from the group consisting of sodium or potassium ferricyanide, sodium or potassium ferricyanide, Nokes reagent (mixture of P<sub>2</sub>S<sub>5</sub> and NaOH), sodium sulfide and sodium hydrosulfide or mixtures thereof which selectively depresses the non-molybdenite fraction and

4. subjecting the molybdenite to froth flotation to recover the enriched molybdenite float.
- 20 2. A process according to claim 1 wherein the organic collector used to produce said copper concentrates is selected from the group consisting of a dithiophosphate, a xanthate and a carbamate or mixtures thereof.
- 25 3. A process according to claim 1 wherein the soluble metal salt is selected from the group consisting of a copper sulfate salt, a zinc sulfate salt and an aluminum sulfate salt or mixtures for a
- 30 4. A process according to claim 1 wherein the principal collector used to produce the copper concentrate is a dithiophosphate; the concentrate is thickened to 16-60 percent solids and treated for period of time with a soluble metal of copper, zinc and aluminum and fuel oil; the pulp treated with a peroxygen compound defined in claim 4 at a pH of 4-8; the thus conditioned pulp subjected to froth flotation using a depressant or depressants as defined in claim 5 and recovering molybdenite from the enriched float.
- 35 5. A process according to claim 4 wherein the concentrate is thickened to 40-60 percent solids and treated for 1-20 minutes with a soluble metal salt before the addition of the peroxygen compound.
- 40 6. A process according to claim 4 wherein 0.5 - 3.0 lbs of a metal salt per ton of concentrate is added.
- 45 7. A process according to claim 6 wherein the soluble metal salt is selected from the group consisting of cupric sulfate, zinc sulfate and aluminum sulfate.
- 50 8. A process according to claim 7, wherein the source of the metal salt is a leach solution containing the metal sulfate.
- 55 9. A process according to claim 4 wherein 0.25-4.0 pounds of H<sub>2</sub>O<sub>2</sub> per ton of concentrate is added.
- 60 10. A process according to claim 4 wherein the depressant is ferrocyanide and/or a mixture of ferrocyanide and ferricyanide.
- 65 11. A process according to claim 4 wherein the depressant is Nokes reagent (a mixture of P<sub>2</sub>S<sub>5</sub>/NaOH).
- 70 12. A process according to claim 4 wherein depressant is Na<sub>2</sub>S and/or NaSH.
- 75 13. A process according to claim 4 wherein the depressant is a mixture of ferrocyanide and Nokes reagent (P<sub>2</sub>S<sub>5</sub>/NaOH).
- 80 14. A process according to claim 4 wherein the collector used to produce the copper concentrate is a dithiophosphate of the type obtained by reacting cresylic acid and P<sub>2</sub>S<sub>5</sub>.

\* \* \* \* \*

UNITED STATES PATENT OFFICE  
CERTIFICATE OF CORRECTION

Patent No. 3,811,569 Dated May 21, 1974

Inventor(s) Joseph Floyd Shirley et al.

It is certified that error appears in the above-identified patent and that said Letters Patent are hereby corrected as shown below:

Inventor's name, page 1, "Edward Frank Caropreso" should read --Frank Edward Caropreso--.

Column 6, claim 3, line 29, "for a" should read --thereof--;

Column 6, claim 4, change claim nos. to read --claim 2-- both occurrences.

Column 2, line 50, "the molybdenite fraction" should read --the non-molybdenite fraction--. (Applicants' error)

Signed and sealed this 17th day of June 1975.

(SEAL)

Attest:

RUTH C. MASON  
Attesting Officer

C. MARSHALL DANN  
Commissioner of Patents  
and Trademarks